

# United States Patent

Reed

[15] 3,661,591

[45] May 9, 1972

## [54] DIAZOTYPE MATERIALS

[72] Inventor: **Peter William Maurice Reed**, Hockley, England

[73] Assignee: **Ozalid Company Limited**, Loughton, Essex, England

[22] Filed: **Mar. 24, 1970**

[21] Appl. No.: **22,391**

## [30] Foreign Application Priority Data

Mar. 28, 1969 Great Britain.....16,418/69

[52] U.S. Cl.....96/91, 96/75

[51] Int. Cl.....G03c 1/52

[58] Field of Search.....96/91, 75

[56]

## References Cited

### UNITED STATES PATENTS

|           |        |                    |       |
|-----------|--------|--------------------|-------|
| 3,525,618 | 8/1970 | Keller et al. .... | 96/75 |
| 2,378,583 | 6/1945 | Schmidt.....       | 96/91 |

Primary Examiner—Norman G. Torchin

Assistant Examiner—John L. Goodrow

Attorney—Cushman, Darby & Cushman

[57]

## ABSTRACT

A diazotype material for use in making copies of X-ray films which comprises a support carrying a light-sensitive layer containing at least one diazonium compound, a coupler and a non-light-sensitive ultra-violet absorber, the ultra-violet absorber being effective in screening out radiation in the range of 3,400 to 4,000 Å, being transparent to all radiation at or above 4,300 Å and being present in an amount such as to give a background absorbance of at least 0.9 at 4,000 Å.

4 Claims, No Drawings

## DIAZOTYPE MATERIALS

It is highly desirable to provide duplicates of silver type X-ray films for the use of those who have to attend the patient and it is essential that such duplicates should show hair line cracks and other fine detail in the original. Hitherto it has only been possible to obtain acceptable duplicates by silver photography and duplicates made in this way are expensive.

Diazotype materials are primarily used for making copies of documents and for such use the primary requirement is high contrast between the bleached and colored areas of the copy. It is possible, however, to obtain some degree of tonal gradation in diazotype copies by inclusion in the light-sensitive layer of a plurality of diazonium compounds having overlapping absorption curves for the radiation to which the material is exposed when making a copy.

The present invention is based upon the discovery that it is possible to produce copies of X-ray films acceptable to the medical profession by using a two-component diazotype material which comprises a support carrying a light-sensitive layer containing at least one diazonium compound, a coupler and a non-light sensitive ultra-violet absorber, the ultra-violet absorber being effective in screening out radiation in the range of 3,400 to 4,000 Å, being transparent to all radiation at or above 4,300 Å and being present in an amount such as to give a background absorbance of at least 0.9 at 4,000 Å.

A two component diazotype material for use in making from microfilms copies from which further copies can be made has been proposed in British Specification No. 1094374. This material contains an ultra-violet absorber which is effective in screening out radiation having a wave length in the range of 3,400–3,900 Å, is transparent to radiation of wave length at and above 4,000 Å, and is present in an amount giving a maximum background absorbance of 0.6 at 4,000 Å.

Experiment has shown that this material produces copies of X-ray photographs which are wholly unacceptable since the required fine detail is totally invisible. The material according to the invention, on the other hand, produces copies which are unsuitable for generating further copies because of the high background absorbance.

One U.V. absorber which can be utilized in the diazotype material according to the invention is 7-diethylamino-4-methyl-coumarin which is on sale as an optical whitening agent under the Registered Trade Mark "Coumalux." Diazotype material containing this U.V. absorber and with the light-sensitive layer supported on a transparent film backing has been found to have, in the bleached and developed condition, an absorbance of 1.52 at 3,400 Å, a peak absorbance of 1.9 at 3,720 Å, an absorbance of 1.18 at 4,000 Å, an absorbance of 0.08 at 4,300 Å and an absorbance of 0.06 at 4,400 Å.

Another example of U.V. absorber which can be used is the coumarin derivative sold by CIBA under the Trade Mark "UVITEX SWR." Diazotype material containing this U.V. absorber in its light-sensitive layer has, in the bleached and developed condition, an absorbance considerably in excess of 2 in the range 3,400–4,000 Å, an absorbance of 0.2 at 4,300 Å and an absorbance of 0.16 at 4,400 Å.

If desired, the light-sensitive layer of the diazotype material according to the invention may be transparent to radiation of wavelength 4,400 Å or more. It will normally include in its light-sensitive layer two or more diazonium compounds having overlapping absorption curves. Preferably the background absorbance of the light-sensitive layer does not exceed 2.0.

The support may normally be a transparent film of, for example, a polyester, such as "Melinex" (Registered Trade Mark) or cellulose acetate because the medical profession prefers to examine X-ray photographs as transparencies. Adequate copies of X-ray films can, however, be produced on diazotype material having a paper support.

The support may, if desired, be pre-treated to facilitate adhesion of the light-sensitive layer. It may also be given a coating of lacquer before application of the light-sensitive layer. Alternatively lacquer may be incorporated in the light-sensitive layer.

Examples of suitable lacquers are cellulose acetate, cellulose acetate propionate, cellulose acetate butyrate, polyvinyl acetate and polyvinyl formal. Fillers, such as finely divided silica, may be added to the lacquer.

Examples of suitable compounds which may be employed are:

p-diethylamino-2-ethoxybenzenediazonium fluoroborate; 2,5-diethoxy-4-morpholinobenzenediazonium fluoroborate; p-diethylaminobenzenediazonium fluoroborate; 1-diazo-4-(N-hydroxyethyl-N-ethylamino)-benzene fluoroborate; 1-diazo-2-ethoxy-4-(N,N-diethylamino)-benzene fluoroborate; 1,diazo-2,5-dimethoxy-4-morpholino-benzene fluoroborate; 1-diazo-4-(N,N-dimethylamino)-benzene fluoroborate; 1-diazo-3-methyl-4-ethylamino-benzene fluoroborate; 1-diazo-2,5-diethoxy-4-morpholino-benzene fluoroborate and 1-diazo-4-(N,N-diethylamino)-benzene fluoroborate.

Examples of suitable couplers are:

2,3-naphthalenediol; naphthalene 2,3-dihydroxy-6-sulphinic acid; resorcinol; 4,4'-dirosorcinol, acetoacetanilide; acetoacet-o-toluidide; chlororesorcinol; N,N-bis-β-hydroxyethyl-2-hydroxy-3-naphthoamide; N-(2'-methylphenyl)-2-hydroxy-3-naphthoamide; N-γ-morpholino-n-propyl-2-hydroxy-3-naphthoamide and N,N-bis-β-hydroxyethyl-2-hydroxy-3-naphthoamide.

The invention will be further illustrated with reference to the following examples:

## EXAMPLE 1

A polyester film (Melinex 'S' Grade) of 0.003 inch thickness was treated with trichloroacetic acid and silica and was then coated with a lacquer which consisted of:

|    |                                                                                                                                                                                                |                                                     |
|----|------------------------------------------------------------------------------------------------------------------------------------------------------------------------------------------------|-----------------------------------------------------|
| 40 | ½ second viscosity Cellulose Acetate Butyrate<br>Polyvinyl Acetate/Polyvinyl Alcohol copolymer<br>dissolved in a mixture of:<br>Toluol<br>74 overproof Industrial Methylated Spirit<br>Acetone | 20.25 g<br>1.08 g<br>49.16 ml<br>11.4 ml<br>39.0 ml |
|----|------------------------------------------------------------------------------------------------------------------------------------------------------------------------------------------------|-----------------------------------------------------|

together with 0.8 grams of finely divided silica (average particle size 10 $\mu$ ).

The lacquer was coated on the polyester film and then dried at approximately 140° C. The coating thickness of the dried lacquer was approximately 0.0003 inch.

The lacquered film was then coated with a layer of light-sensitive material which consisted of:

|    |                                                                                                                                                                                                                                                                                                                                 |                                                                      |
|----|---------------------------------------------------------------------------------------------------------------------------------------------------------------------------------------------------------------------------------------------------------------------------------------------------------------------------------|----------------------------------------------------------------------|
| 55 | Tartaric Acid<br>Resorcinol<br>N-(2'-methylphenyl)-2-hydroxy-3-naphthoamide<br>N,N-bis-β-hydroxyethyl-2-hydroxy-3-naphthoamide<br>1-diazo-4-(N,N-diethylamino)-benzene fluoroborate<br>1-diazo-2-ethoxy-4-(N,N-diethylamino) benzene<br>fluoroborate<br>1-diazo-2,5-diethoxy-4-morpholino benzene<br>fluoroborate<br>"Coumalux" | 2.0 g<br>0.3 g<br>0.4 g<br>0.5 g<br>0.6 g<br>0.6 g<br>0.3 g<br>1.2 g |
| 60 | dissolved in:<br>Methyl ethyl ketone<br>74 overproof Industrial Methylated Spirit                                                                                                                                                                                                                                               | 50 ml<br>50 ml                                                       |

and then dried at about 110° C. The coating weight of the sensitizer was adjusted to give a maximum optical transmission density of 1.5. The background absorbance of the material was approximately 1.06.

This diazotype material gives good reproduction of X-ray films of the silver type.

## EXAMPLE 2

The procedure of Example 1 was repeated except that an equivalent amount of cellulose acetate propionate was utilised in the lacquer in place of the cellulose acetate butyrate.

The background absorbance of the diazotype material was approximately 1.06.

## EXAMPLE 3

The lacquer and the sensitizer set out in Example 1 were mixed together in the ratio of 1 : 1 by volume and coated on the polyester film. After drying at approximately 120° C., the coating had a thickness of approximately 0.0003 inch. The background absorbance was greater than 0.9.

## EXAMPLES 4 - 6

The procedure set out in Examples 1 to 3 were repeated with the "Coumalux" replaced by the ultra-violet absorbing composition sold by CIBA under the Trade Mark "UVITEX 15 SWR."

Good copies of X-ray films of the silver type were again obtained.

In the following Examples 7-9, Example 1 was repeated using the following light-sensitive compositions dissolved in the above stated solvent mixture:

## EXAMPLE 7

|                                                                     |       |
|---------------------------------------------------------------------|-------|
| Tartaric acid                                                       | 2.0 g |
| Resorcinol                                                          | 0.3 g |
| N,N-bis- $\beta$ -hydroxyethyl- $\gamma$ 2-hydroxy-3-naphthoamide   | 0.4 g |
| N-(2'-methylphenyl)-2-hydroxy-3-naphthoamide                        | 0.5 g |
| 1-diazo-4-(N-hydroxyethyl-N-ethylamino)-benzene fluoroborate        | 0.6 g |
| 1-diazo-2-ethoxy-4-N-hydroxyethyl-N-ethylamino-benzene fluoroborate | 0.6 g |
| 1-diazo-2,5-dimethoxy-4-morpholino-benzene fluoroborate             | 0.3 g |
| "Coumalux"                                                          | 1.2 g |

## EXAMPLE 8

|                                                           |       |
|-----------------------------------------------------------|-------|
| Citric acid                                               | 2.0 g |
| Resorcinol                                                | 0.3 g |
| N-(2'-methylphenyl)-2-hydroxy-3-naphthoamide              | 0.5 g |
| N- $\gamma$ -morpholino-n-propyl-2-hydroxy-3-naphthoamide | 0.4 g |

|                                                        |       |
|--------------------------------------------------------|-------|
| 1-diazo-4-(N,N-dimethylamino)-benzene fluoroborate     | 0.6 g |
| 1-diazo-3-methyl-4-ethylamino-benzene fluoroborate     | 0.6 g |
| 1-diazo-2,5-diethoxy-4-morpholino-benzene fluoroborate | 0.3 g |
| "Coumalux"                                             | 1.4 g |

## EXAMPLE 9

5 10

|                                                            |          |
|------------------------------------------------------------|----------|
| Methyl ethyl Ketone                                        | 50.5 mls |
| Industrial Methylated Spirit                               | 50.0 mls |
| Tartaric acid                                              | 2.0 g    |
| Resorcinol                                                 | 0.3 g    |
| N-(2'-methylphenyl)-2-hydroxy-3-naphthoamide               | 0.4 g    |
| N,N-bis- $\beta$ -hydroxyethyl-2-hydroxy-3-naphthoamide    | 0.5 g    |
| 1-diazo-4-(N,N-diethylamino)-benzene fluoroborate          | 0.6 g    |
| 1-diazo-2-ethoxy-4-(N,N-diethylamino)-benzene fluoroborate | 0.6 g    |
| 1-diazo-2,5-diethoxy-4-morpholino-benzene fluoroborate     | 0.3 g    |
| "Coumalux"                                                 | 1.2 g    |

What I claim as my invention and desire to secure by Letters 25 Patent is:

1. A diazotype copying material for use in making duplicates of silver halide X-ray films, said material comprising a support and, carried upon said support, a light-sensitive layer containing three diazonium compounds having overlapping absorption curves, a coupler and a nonlight sensitive ultra-violet absorber consisting essentially of 7-diethylamino-4-methyl coumarin, said light-sensitive layer having a background absorbance of at least 0.9 at 4,000 Å.
2. A diazotype copying material as claimed in claim 1, whereon the background absorbance at 4,000 Å of the light-sensitive layer does not exceed 2.0.
3. A diazotype copying material as claimed in claim 1, wherein the support is a transparent film.
4. A copying material as claimed in claim 1, wherein the 40 diazonium compounds are 1-diazo-4-(N,N-diethylamino)-benzene fluoroborate, 1-diazo-2-ethoxy-4-(N,N-diethylamino)-benzene fluoroborate and 1-diazo-2,5-diethoxy-4-morpholino-benzene fluoroborate.

\* \* \* \* \*

45

50

55

60

65

70

75